

## UNITED STATES PATENT OFFICE

2,511,250

STABILIZED EXTREME PRESSURE  
LUBRICANTS

Jack S. Fawcett, Tarentum, Pa., assignor to Gulf  
Research & Development Company, Pittsburgh,  
Pa., a corporation of Delaware

No Drawing. Application November 14, 1947,  
Serial No. 786,151

6 Claims. (Cl. 252—33)

1

This invention relates to improved oil compositions and more particularly to stabilized extreme pressure lubricants.

Extreme pressure lubricants are employed for lubricating bearings and gears operating under high pressures. They are also employed to carry off excess heat generated and to lessen the friction created during metal cutting operations. While plain mineral oils are satisfactory for removing heat during severe cutting operations, they do not have a sufficiently high film strength for the maintaining of a lubricating film between the tool, die or roll and the metal being processed, nor do they have a sufficiently high film strength to prevent seizure and scoring of metallic surfaces movably contacting each other under extreme pressures. The film strength or load carrying capacity of plain mineral oils has been enhanced by the addition of various extreme pressure agents containing either a halogen or sulfur, or mixtures thereof. Although oils containing extreme pressure agents such as these have good load carrying characteristics, they have a serious disadvantage in that a halogen or sulfur in oils lead to the formation of a stain on ferrous and non-ferrous alloys. Furthermore, in the presence of moisture, ferrous and non-ferrous alloys become severely corroded when contacted with an oil composition containing a halogen or sulfur.

It is an object achieved by this invention to provide an improved extreme pressure lubricant which effectively inhibits the staining and/or corrosion of ferrous and non-ferrous alloys.

It is a further object achieved by this invention to provide an improved extreme pressure lubricant in which corrosive properties of the extreme pressure lubricant are inhibited without deleteriously modifying the desirable properties of the extreme pressure lubricant.

I have found that a lubricant containing an extreme pressure agent normally tending to corrode ferrous and non-ferrous alloys can be made substantially non-corrosive to said alloys by incorporating in the extreme pressure lubricant a small amount, sufficient to inhibit the corrosive properties, of the triethanolamine salt of the oil soluble petroleum sulfonic acids. The amount of the triethanolamine salt of the oil soluble petroleum sulfonic acids which may be incorporated in the composition of my invention varies between about 0.05 and about 1.0 per cent by weight, the exact amount in any particular case depending upon the severity of the conditions to which the composition is subjected and upon the

2

amount and the nature of the extreme pressure agent contained in the lubricant.

In addition to the extreme pressure agent and the triethanolamine salt of the oil soluble petroleum sulfonic acids, the finished extreme pressure lubricant in accordance with my invention may also contain other "additive" agents including viscosity index improvers, such as high molecular weight polymers of isobutylene and the polymers of methacrylic esters; pour point depressants, such as a condensation product of chlorinated wax and naphthalene and a condensation product of chlorinated wax and phenol followed by further condensation of this reaction product with organic acids; detergents, such as nickel naphthenate, metal salts of ethyl hexyl salicylate, and metal salts of alkyl substituted phenol sulfides; and foam inhibitors, such as organo-silicon oxide condensation products, organo-silico condensation products, and organo-germanium oxide condensation products.

In preparing the stabilized extreme pressure lubricants in accordance with my invention, the triethanolamine salt of the oil soluble petroleum sulfonic acids may be incorporated in the extreme pressure lubricant, according to several embodiments. For example, the triethanolamine salt per se may be added to the lubricant, or the triethanolamine salt may be produced directly in the extreme pressure lubricant by separately adding triethanolamine and the oil soluble petroleum sulfonic acids. According to another embodiment, oil concentrates containing relatively high concentrations of the triethanolamine salt of the oil soluble petroleum sulfonic acids may be first prepared and the desired concentration obtained in the extreme pressure lubricant by adding the concentrate thereto. The latter method is advantageous in that the oil concentrate is less viscous and can be more readily dissolved in the extreme lubricant.

In preparing the triethanolamine salt of the oil soluble petroleum sulfonic acids for use in accordance with my invention, I prefer to employ the oil soluble petroleum sulfonic acids generally referred to as "mahogany acids." These acids, together with the water soluble "green acids," are produced during the acid refining of petroleum distillates with sulfuric acid. There are two general methods employed in recovering the "mahogany" acids. The first method involves selectively removing the acids by adsorbents or by solvents such as the lower mono-basic alcohols. The second method involves salting out the acids with inorganic salts or bases. These methods are

well-known and have been described in detail by Carleton Ellis on page 1070 of volume 2 of "The Chemistry of Petroleum Derivatives," Reinhold Publishing Corporation, New York, 1937 (second printing 1945). The particular petroleum sulfonic acids used in preparing the triethanolamine salt in accordance with the procedure hereinafter set forth were obtained by acidifying an aqueous suspension of the sodium salt of the oil soluble petroleum sulfonic acids with hydrogen chloride and subsequently extracting the acids with a suitable solvent such as ethyl ether. The average molecular weight of these acids was about 400 as determined by the neutralization equivalent.

The triethanolamine salt of the oil soluble petroleum sulfonic acids in the tests hereinafter described consisted of an oil concentrate of the triethanolamine salt of the oil soluble petroleum sulfonic acids and was obtained by the following procedure:

50 grams of a 50/50 mixture of mineral oil and oil soluble petroleum sulfonic acids and 9.2 grams of triethanolamine, each at room temperature, were placed in a reaction vessel. The contents of the reaction vessel were then stirred for about an hour. The reaction which takes place is an exothermic reaction so that the temperature of the contents of the reaction vessel rose to about 135° to 140° F. during the reaction period. The reaction mass was a dark brown viscous material about the consistency of a medium petrolatum. The reaction mass consisted of an oil concentrate containing about 60 per cent by weight of the triethanolamine salt of the oil soluble petroleum sulfonic acids.

In the practice of my invention any suitable lubricating oil base, whether it be derived from a paraffinic, naphthenic, or mixed base crude, may be employed. The extreme pressure lubri-

agents may be mentioned the chlorinated derivatives of paraffin wax, kerosene, aromatic petroleum fractions, and coal tar solvents (naphthalene tetrachloride). A chlorine-containing extreme pressure agent is ordinarily employed in an amount sufficient to produce a chlorine content in the extreme pressure lubricant between about 1 and about 10 per cent by weight. Thus, when an extreme pressure agent containing 40 per cent of chlorine is used, the agent may be employed in the oil in an amount between about 2.5 and 25 per cent by weight.

10 The advantages to be obtained by the use of the triethanolamine salt of the oil soluble petroleum sulfonic acids according to my invention are illustrated in the following specific tests:

15 In these tests a highly refined light naphthenic Texas oil of 100 S. U. V. at 100° F. and No. 2 N. P. A. color having a gravity of 24° A. P. I. was used. The effect of a sample of this oil containing 20 10 per cent by weight of a chlorinated liquid hydrocarbon containing about 40 per cent by weight of chlorine on polished hot rolled S. A. E. 1020 steel strips 6" x 1/2" x 1/8" in the presence of and in the absence of distilled water was compared with the effect of another sample containing 25 10 per cent by weight of a chlorinated liquid hydrocarbon containing about 40 per cent by weight of chlorine and 0.5 per cent by weight of an oil concentrate containing 60 per cent by weight of the triethanolamine salt of the oil soluble petroleum sulfonic acids.

30 In carrying out these tests, the hot rolled steel strips were half immersed in the respective oil samples in separate glass containers. The oil samples were maintained at a temperature of 122° F. In the following table there are shown the compositions tested and a comparison of the 35 respective results showing the number of hours before corrosion began to occur.

|                                                                                                                                                                                                              | Without Water                          | With 5% Distilled Water                |
|--------------------------------------------------------------------------------------------------------------------------------------------------------------------------------------------------------------|----------------------------------------|----------------------------------------|
| Sample No. 1:<br>90% 100/2 Texas oil, 10% Chlorinated hydrocarbon (40% chlorine).                                                                                                                            | Slight stain after 72 hours, @ 122° F. | Severe rust after 4-5 hours, @ 122° F. |
| Sample No. 2:<br>89.5% 100/2 Texas oil, 10% Chlorinated hydrocarbon (40% chlorine), 0.5% Oil concentrate of the triethanolamine salt of the oil soluble petroleum sulfonic acids (60% triethanolamine salt). | No rust after 92 hours, @ 122° F.      | No rust after 92 hours, @ 122° F.      |

cant to which the triethanolamine salt of the oil soluble petroleum sulfonic acids, according to my invention, may be added may be prepared by incorporating into a lubricating oil having a viscosity between the approximate limits of 50 S. U. S. and 1200 S. U. S. at 100° F. an extreme pressure agent containing a halogen or sulfur, or mixtures thereof. The extreme pressure agent is added to the lubricating oil in an amount sufficient to impart extreme pressure characteristics and normally to impart corrosive properties. This amount may vary between 1 and 25 per cent by weight, but in any particular case the amount employed depends upon the severity of the conditions under which the oil is to be used, and upon the amount of halogen or sulfur in the extreme pressure agent. Generally the amount of halogen or sulfur in an extreme pressure compound is between the approximate limits of 5 and 75 per cent.

70 My invention is particularly applicable to extreme pressure lubricants containing corrosive chlorine compounds, such as chlorinated aliphatic or aromatic hydrocarbons. Among the more common chlorinated extreme pressure

75 The data given in the table demonstrate the remarkable effect obtained when 0.5 per cent of an oil concentrate of the triethanolamine salt of the oil soluble petroleum sulfonic acids is added to a normally-corrosive extreme pressure lubricant. In sample No. 1, it will be noted that slight stain appeared on the steel strip even in the absence of water after immersion in the oil for 72 hours. It will be further noted that severe rusting occurred after only 4 to 5 hours' immersion in the oil in the presence of 5 per cent distilled water. When only 0.5 per cent by weight of the oil concentrate of the triethanolamine salt of the oil soluble petroleum sulfonic acids was incorporated in the oil, in accordance with sample No. 2, no rusting occurred after 92 hours either in the presence of or in the absence of water.

While my invention has been described above with reference to various specific examples and embodiments, it will be understood that the invention is not limited to the illustrated examples and embodiments and may be variously practiced within the scope of the following claims.

I therefore claim:

1. A stabilized extreme pressure lubricant consisting predominantly of a lubricating oil, an extreme pressure agent consisting of a halogenated hydrocarbon in an amount sufficient to impart extreme pressure characteristics and normally to impart corrosive properties, and a small amount, sufficient to inhibit said corrosive properties, of the triethanolamine salt of the oil soluble petroleum sulfonic acids.

2. A stabilized extreme pressure lubricant consisting predominantly of a lubricating oil, an extreme pressure agent consisting of a chlorinated hydrocarbon in an amount sufficient to impart extreme pressure characteristics and normally to impart corrosive properties, and a small amount, sufficient to inhibit said corrosive properties, of the triethanolamine salt of the oil soluble petroleum sulfonic acids.

3. A stabilized extreme pressure lubricant consisting predominantly of a lubricating oil, 1 to 25 per cent by weight of an extreme pressure agent consisting of a chlorinated hydrocarbon, and about 0.05 to about 1.0 per cent by weight of the triethanolamine salt of the oil soluble petroleum sulfonic acids.

4. A stabilized extreme pressure lubricant consisting predominantly of a lubricating oil, an extreme pressure agent consisting of a chlorinated hydrocarbon in an amount sufficient to produce a chlorine content in the extreme pressure lubricant between about 1 and about 10 per cent

by weight, and about 0.05 to about 1.0 per cent by weight of the triethanolamine salt of the oil soluble petroleum sulfonic acids.

5. A stabilized extreme pressure lubricant consisting of about 74 to 97.5 per cent by weight of a lubricating oil, about 2.5 to 25 per cent by weight of a chlorinated hydrocarbon containing about 40 per cent chlorine, and about 0.05 to about 1.0 per cent by weight of the triethanolamine salt of the oil soluble petroleum sulfonic acids.

6. A stabilized extreme pressure lubricant consisting of 89.5 per cent by weight of a lubricating oil, 10 per cent by weight of a chlorinated hydrocarbon containing about 40 per cent of chlorine, and 0.5 per cent by weight of an oil concentrate containing about 60 per cent by weight of the triethanolamine salt of the oil soluble petroleum sulfonic acids.

JACK S. FAWCETT.

#### REFERENCES CITED

The following references are of record in the file of this patent:

#### UNITED STATES PATENTS

| Number    | Name           | Date          |
|-----------|----------------|---------------|
| 2,049,043 | Birkby         | July 28, 1936 |
| 2,268,603 | McNulty et al. | Jan. 6, 1942  |
| 2,298,636 | Frutton        | Oct. 13, 1942 |
| 2,333,206 | Sloan          | Nov. 2, 1943  |
| 2,392,891 | Wallace et al. | Jan. 15, 1946 |